

# UNITED STATES PATENT OFFICE.

CHARLES KNOX HARDING, OF CHICAGO, ILLINOIS.

## ELECTRIC SPARK-PLUG.

1,296,076.

Specification of Letters Patent.

Patented Mar. 4, 1919.

No Drawing.

Application filed June 3, 1918. Serial No. 238,068.

To all whom it may concern:

Be it known that I, CHARLES KNOX HARDING, a citizen of the United States, and a resident of Woodlawn, city of Chicago, county of Cook, State of Illinois, have invented certain new and useful Improvements in Electric Spark-Plugs, of which the following is a specification.

The object of this invention is to produce an improved electric spark plug having an improved ceramic structure for carrying and insulating from each other the metallic conducting electrodes which are usually carried in a suitable metal shell detachably screwed into an opening in the wall of internal combustion engines.

This invention relates particularly to a new class of non-carbonizing spark plugs which are required to operate at an extremely high temperature, such as described in my United States Patent No. 1,272,431, July 16th, and No. 1,275,020, Aug 6, 1918.

The insulating material most commonly used for spark plug insulators is porcelain and its defects at high temperatures are well known. Among them may be mentioned its low, dielectric insulating properties at high temperatures, and this I believe is caused by the heterogeneous character of the highly acid and extremely basic oxids, such as silica,  $\text{SiO}_2$  on the one end and alkalis as potash  $\text{K}_2\text{O}$  at the extreme opposite end of the series of which all vitreous earthenware insulators have heretofore been made.

I have discovered that the refractory oxids of which a much improved spark plug insulating structure is formed should be neutral, or very nearly neutral, and not be subject to form eutectic compounds of widely varying basic and acid slag-forming and easily electrolyzed character. The group of suitable neutral oxids will be specifically described hereinafter.

The theoretical assumption—that viscous fused silica the vitrified as distinguished from the crystalline form is when cold composed of very large condensed aggregates of enormous molecular weight, each consisting of a large number of silica molecules polymerized and forming a large molecular compound unit carrying equally balanced positive and negative charges or electrons—and that these polymerids gradually break up into smaller masses with comparative small

increase of temperature without any marked 55 change in the physical character of the mass or structure of which they form a part, this theory is confirmed by the fact that ceramic bodies containing fused silica such as porcelain, earthenware, etc., show an almost 60 constant increase of electric conductivity with increase of temperature so that an increase of temperature of as little as 25 or 50 degrees Fahr. will double the conductivity—presumably by doubling the number of 65 polymerized charge-carrying masses—and the regular falling to half the value of the resistance with each equal addition of heat so that from any temperature—the increase through six of these intervals would reduce 70 the insulating value proportionately to the sixth power of two, or by sixty-four times—these changes go on in all ceramic structures containing polymerized silica molecules several hundred degrees below any fusing or softening point of the body of which the insulator is made. These considerations have aided 75 in the discovery of my improved spark plug in which the insulating structure is formed from oxids of chemically neutral elements 80 of high atomic weight, i. e., from 90 to 232, so that insulators containing a given weight of oxids contain only from one-half to one-fourth as many molecules as would be the case if their mass was made up of oxids of 85 aluminum or silicon.

The most neutral of the known earth oxids is lanthanum oxid. The dydimiums are next which are almost equally neutral and do not tend to flux or form silicates 90 while the next closest of the most neutral group on the one side is zirconium oxid and thorium oxid on the other which are almost neutral but will form silicates. My experiments have demonstrated that lanthanum 95 oxid and compounds thereof when forming the principal constituents of refractory ceramic insulating structures, such as spark plug insulators, produce an improved insulator superior to anything heretofore known 100 or used for the purpose where the insulator was operated at high temperature.

A careful examination of all the non-combustible insulators known or used up to the year A. D. 1915, including steatite, mica, 105 and all kinds of porcelain and earthenware disclosed that all contained what I consider to be a great excess of silica, silicon dioxid.

This silica or flint necessarily carries into the structure too much of its friable, frangible, fragile and other undesirable properties for a body required to withstand sudden and extreme changes of temperature.

The object of my invention was to overcome the defects attributable to silica. I have therefore endeavored to discover or devise a new insulating body as free as possible 10 from silica, and my invention is therefore that of a new and improved spark plug insulator characterized by the absence of a substantially objectionable content of silica.

The potter's art for more than a thousand 15 years has been based on silica and clay—a double silicate of aluminum—but I have by going outside this art produced scores of different refractory ceramic structures containing no clay or aluminum and no silica 20 in any form.

The preferred substance from which to construct the most desirable spark plug insulator, so far as I am at present aware, is one containing an excess of lanthanum oxide 25 over and above any lanthanum compound it may contain and in excess of a varying quantity from 10 to 40 per cent. of lanthanum phosphate which it may contain without disadvantage. The highest purity 30 is not required and oxides of the other neutral elements may be added or left in the partly refined lanthanum compound, which is most conveniently obtained from the mineral, monazite, which usually contains about 35 90% of phosphates of the cerite group of rare earths, from which when the twenty-eight parts of phosphoric acid is removed there remains about 62% of the oxide of praseodymium, cerium, neodymium and lanthanum by what is known as the hydrated sulfate method of separation. Lanthanum hydrated sulfate  $\text{La}_2(\text{SO}_4)_3 \cdot 9(\text{H}_2\text{O})$ , which is by far the least soluble of this group of hydrated sulfates, can be separated in one or 40 two treatments of sufficient purity for use in my improved spark plug insulator. The mixed anhydrous sulfates produced by heating until all the water and excess acid is driven off, is dissolved in about eight parts 45 ice water and then gradually heated until the hydrates form; the various hydrates have varying solubility in the order named above; that is, praseodymium is about seven times as soluble as lanthanum, the hydrated sulfate of cerium  $\text{Ce}_2(\text{SO}_4)_3 \cdot 8(\text{H}_2\text{O})$  about 50 five times as soluble, and neodymium about three and a half times as soluble, so that the first of the precipitate is largely the lanthanum salt. At a little higher temperature 55 the precipitate contains more neodymium, while at a still higher temperature the cerium will become less soluble and considerable cerium will separate with the precipitate. I have not been able to determine 60 as yet exactly what is the best proportion of 65

these rare earth oxides for a spark plug insulator, but experiments indicate a certain amount of both cerium and dysmum oxides is desirable, and it reduces the cost of manufacture to include them in the body of the 70 insulator.

Thorium oxide should not be present in all parts of the insulator in excess as its ionizing effect tends to reduce the dielectric resistance of a film of air at the surface of the 75 insulator.

Most of the processes of the potter's art for forming earthenware structures depending on capillary and colloidal water shrinkage to draw the body into a dense compact 80 mass—cannot be employed with lanthanum—or neutral rare earth oxides—but mixtures of such oxides containing no clay may be formed to the desired shape by so-called dry forming; that is compressing slightly moist materials in steel molds under very heavy 85 pressure.

Finely ground calcined lanthanum—with air dry lanthanum phosphate and 6 to 12 per cent. gelatinous lanthanum hydrate— 90 may be subjected to a high pressure in a metal die and formed into a very compact structure—that will not check in air drying—and may be fired to a very high temperature above Segar cone 20 without injury.

If difficulty is met in reducing the porosity of the formed insulator to the required density—it may be rendered dense and impervious—by impregnating the body with a 100 strong solution of soluble salts of the suitable earths—nitrate, chlorid, etc., of zirconium or the rare earth elements—then drying and refiring to some attainable temperature—eutectic mixtures—of the oxides 105 and phosphates of the rare earths may be formed that will vitrify sufficiently at temperatures between cone 16 and 20.

This process may be varied by saturating the insulator at any stage where it remains 110 to any extent pervious with acid solution of earthy oxides containing excess phosphoric acid—or alternate applications of nitrates which leave only difficultly vitrifiable oxides deposited in the structure may be followed 115 by acid solutions containing an excess of phosphoric acid—which react during the second successive firing to form readily vitrifiable compounds at readily attainable temperatures.

My new process enables insulating structures to be produced of the desired density—of very refractory materials and of great mechanical strength. It enables insulators to be produced having all of the desirable characteristics of the old silicate materials and allows the elimination of objectionable elements and their objectionable characteristics, and the successful employment of the most neutral, though refractory and other- 120 125 130

wise most desirable rare earth oxids of thorium, zirconium, lanthanum, etc.

Ceramic insulators can thus be constructed exclusively from oxids of only the tri-valent and tetra-valent elements and free from easily electrolyzed and slag forming mono-valent alkali elements or the highly basic di-valent elements.

Zirconium oxide is at present the cheapest of the suitable neutral earth oxids and I have manufactured many refractory spark plug insulating structures containing 60 to 70% commercial zirconia that have proved in actual use over many months to withstand the conditions of service where the best grades of porcelain fail. Zirconia insulators have an insulating resistance when cold about 100 times less than cold porcelain or silicates, but are much better than porcelain when hot, and for voltages less than 10,000 to 11,000 volts will probably prove satisfactory where an inexpensive device is required.

Having described my invention, what I claim is:—

- 25 1. An electric spark plug having an improved structure for supporting and insulating the electrodes characterized by being non-fragile, resistant to sudden changes of temperature and having high dielectric resistance when hot, consisting of a ceramic structure comprising zirconium and thorium compounds.
- 30 2. An electric spark plug having a new insulating structure of great mechanical strength and infrangibility under sudden variations of temperature and high electric insulating resistance at high temperature consisting of a ceramic structure comprising

zirconium compounds as its principal constituent.

3. A new electric spark plug having an insulator consisting of a ceramic structure having great mechanical strength and heat resisting properties and high dielectric insulating resistance at high temperatures containing only the desirable neutral earth oxide such as lanthanum and characterized by the absence of objectionable silica.

4. A new electric spark plug having an insulator having great mechanical strength and heat resisting properties and high dielectric insulating resistance at high temperatures, consisting of a ceramic structure composed of mixtures of desirable neutral earth oxides such as zirconia and characterized by the absence of the element silicon in any of its forms.

5. An improved spark plug having an insulator composed exclusively of neutral tri-valent and tetra-valent earth oxids, such as lanthanum, thorium, zirconium and didymium.

6. The improved electric spark plug having an insulator distinguished from known insulators by its composition being practically free from alkalis and silica.

7. An electric spark plug having an improved insulator consisting of a ceramic structure composed principally of neutral tri-valent and tetra-valent earth oxid compounds and including cerium compounds.

In testimony whereof, I have signed my name to this specification this the 31st day of May, A. D. 1918.

CHARLES KNOX HARDING.